

Feb. 21, 1956

6  
**F. J. MANN**  
METAL-IMPREGNATED HEATING RODS FOR ELECTRIC  
FURNACES AND METHOD OF MAKING SAME  
Filed Dec. 27, 1952

2,735,881

FIG. I



FIG. 2



INVENTOR

FRANZ JOSEPH MANN

BY

ATTORNEY

1

2,735,881

**METAL-IMPREGNATED HEATING RODS FOR ELECTRIC FURNACES AND METHOD OF MAKING SAME**

Franz Josef Mann, Erlangen, Germany, assignor to Siemens-Planiawerke Aktiengesellschaft für Kohlefabrikate, Metingen bei Augsburg, Germany, a corporation of Germany

Application December 27, 1952, Serial No. 328,187

Claims priority, application Germany January 25, 1952

16 Claims. (Cl. 13—25)

This invention relates to resistor rods provided with enlarged terminal ends, for use in electric furnaces having relatively thick walls, and is particularly concerned with resistor rods having formed porous bodies preferably made of silicon carbide or of metallic powder or a powder mixture or metal compositions, alloys, or heat-resisting oxides.

In order to keep the temperature at the terminal ends of the resistor rods as low as possible, such terminal ends were in prior structures carried to the outside of the furnace walls, so as to provide for effective cooling. However, the furnaces must be equipped with relatively thick walls so as to keep thermal losses low; and, if the contact with the resistor rods is to be made outside of the furnace walls, they must be provided with very long terminal ends, resulting in increased cost and insufficient utilization of the portions thereof which extend through the furnace walls. It has therefore been proposed to keep the terminal ends of the resistor rods relatively short, as compared with the wall thickness of the furnace, and to dispose in the furnace walls the contact members or heads for engagement with the associated terminal ends of the resistor rods. Resistor rods are used having thickened terminal ends which have, due to their greater cross-sectional areas, a considerably lower resistance than the heating portions thereof. The contacting surfaces of the resistor rods were provided with a conductive metallic coating in order to keep the transition resistance at the contacting surfaces between the contact members and the associated terminal ends of the resistor rods as small as possible.

One object of the invention is to reduce the cross-sectional areas of the terminal ends of the resistor rods so as to increase the heat capacity of the corresponding furnace by providing an increased number of resistor rods closely adjacent one another.

The thickened terminal ends of the resistor rods are, in accordance with the invention, impregnated with metal that flows in melted condition so as to obtain, with reduced cross-section, the necessary electrical conductivity and to keep low the temperature produced by the current flow in such terminal ends. The metal penetrates deep into the pores of the portion of the resistor rods that is to be impregnated and fills the hollow spaces throughout the entire cross-sectional area thereof. However, this metallic impregnation can be accomplished only if the corresponding formed body exhibits the required porosity, as is the case, e. g., with formed bodies of silicon carbide.

Suitably formed bodies having the desired porosity may also be produced metallurgically from powders of high-melting metals and heat-resisting oxides. Among such metals is molybdenum intermixed with a nonconductive material such as zirconium oxide or other oxides of the alkaline earth metals.

The use of porous formed resistor rod bodies permits, as an advantageous feature, to provide upon the heating

2

portion thereof a thin protective coating which is insensitive to high temperatures and protects it against chemical attacks of the hot furnace gases.

Such a protective coating may be formed from initial substances which are in melted condition or in solution adapted to penetrate into the pores of the rod and which may by subsequent thermal or chemical treatment be transformed to compositions yielding a dense, chemically inert but heat-resisting coating. Aluminum oxide spinell may be mentioned as a suitable composition of this kind that may be formed by the protective coating.

The radial surfaces of the terminal ends of the resistor rods facing the heating compartment of the furnace are suitably also provided with a protective coating such as is formed on the heating portion thereof.

As already mentioned, the formed body of the resistor rod must have a certain porosity as a requirement for the metallic impregnation of the terminal ends as well as for the anchoring of the protective layer or coating on the surface of the heating portion thereof. The resistor rod is for this purpose made as a unitary and integral body having the terminal ends and also the heating portion formed of the same raw material and in the same production process.

It would appear feasible in the case of resistor rods made metallurgically of powders comprising metals and oxides to enrich the terminal portions metallurgically from the start. However, since the corresponding formed bodies are made by molding or pressing together the various powders prior to the sintering, there will result difficulties in introducing different powder mixtures for the different portions of the bodies into the corresponding mold.

In accordance with a further feature of the invention, the heating portion and also the terminal portions of the resistor rods are made of the identical basic or raw material having a porosity which permits impregnation with metals that flow in melted condition, and which also permits penetration of certain initial substances to form the protective coating.

An example of the invention will now be described with reference to the accompanying drawings, in which

Fig. 1 shows an embodiment of the new resistor rod in part sectional and part elevational view; and

Fig. 2 indicates a portion of a furnace wall in section, also showing in elevation the terminal portion of a resistor rod, and in sectional view the contact head or member associated therewith.

The new resistor rod, as shown in Fig. 1, comprises a formed silicon carbide body having thickened terminal portions 1 at the opposite ends of a heating portion 2. The axially outwardly facing walls of the terminal portions 1 are cone-shaped so as to increase the contact surfaces formed thereby. These terminal portions 1 are impregnated with metallic silicon throughout their entire cross-sectional areas. The silicon is introduced in molten flowing condition by the application of pressure so as to penetrate into the pores of the terminal portions.

The heating portion 2 is provided with a protective layer of aluminum oxide spinell which is anchored in the pores. This protective layer or coating 3 also extends over the radially extending inner walls of the terminal portions 1 which face the heating compartment of the furnace.

In Fig. 2 numeral 4 indicates part of the furnace wall. Current is conducted to the resistor rod 1/2 over the contact head or member 5 made of graphite or suitable metal and provided with a duct 6 for the circulation of a cooling fluid. Numeral 7 indicates the current-supply terminal which is secured on the head 5 by a clamp 8.

A spring (not shown) is provided which extends from the furnace wall to press the contact head 5 against the associated terminal portion of the resistor rod. The contact head 5 and the terminal portion 1 of the resistor rod are disposed inside of a tubular insulating member 9 which is lined with an asbestos tubing 10.

The opposite right hand terminal portion of the heating rod (not shown in Fig. 2) is secured and is supplied with current by means similar to those shown in connection with the illustrated left hand portion thereof.

I claim:

1. A resistor rod for an electric furnace comprising an elongated body made of porous material and forming a centrally axially extending rodlike heating portion and an enlarged terminal portion at each end of said heating portion which is integral therewith, said enlarged terminal portions being impregnated with metal throughout their respective cross-sectional areas and having due to such impregnation a specific resistance which is lower than that of said heating portion.

2. The heating rod as defined in claim 1, having a body made of silicon carbide.

3. The heating rod as defined in claim 1, having a body made of powdered material comprising metal and metal oxide components.

4. The heating rod as defined in claim 2, comprising a protective coating carried by said heating portion.

5. The heating rod as defined in claim 2, wherein said terminal portions are impregnated with metallic silicon.

6. The heating rod as defined in claim 1, wherein the axially outwardly facing ends of said enlarged terminal portions are cone-shaped.

7. The heating rod as defined in claim 4, comprising a protective coating carried by the axially inwardly facing walls of said enlarged terminal portions.

8. The method of making a resistor rod for an electric furnace having an elongated body exhibiting a centrally axially extending rodlike heating portion and an enlarged terminal portion at each end of said heating portion, said method comprising the following steps, namely, taking a raw material and shaping it to form said body integrally therefrom, said integral body being a porous body, and impregnating said enlarged terminal portions with metal throughout the entire cross-sectional areas thereof, said enlarged terminal portions having due to said impregnation a specific resistance which is lower than that of said heating portion.

9. The method defined in claim 8, comprising the step of providing on said heating portion a protective coating which is anchored in the pores thereof.

10. The method defined in claim 9, comprising the step of providing on the axially inwardly facing walls of said terminal portions a protective coating which is anchored in the pores thereof.

11. The method defined in claim 10, wherein said raw material is silicon carbide and wherein said metal impregnation is metallic silicon and wherein said protective coating is formed by aluminum oxide spinel.

12. In the art of producing for use in electric furnaces resistor rods comprising an elongated body having a centrally axially extending rodlike heating portion and an enlarged terminal portion at each end of said heating portion, the method of making such resistor rod comprising the following steps, namely, taking raw material and forming said body integrally therefrom, said integral body exhibiting a porosity adapting it for impregnation by a molten metallic material, impregnating said enlarged terminal portions with said metallic material throughout their entire cross-sectional areas by the application of pressure, and applying to said heating portion and to the axially inwardly facing walls of said enlarged terminal portions a material to form a protective coating thereon.

13. The method defined in claim 12, wherein said raw material is silicon carbide.

14. The method defined in claim 12, wherein said raw material is a powder comprising metal and metal oxide components.

15. The method defined in claim 12, wherein said raw material is molybdenum intermixed with nonconductive oxide.

16. In an electric resistance furnace having a wall forming a heating chamber, a resistor body comprising an elongated rodlike heating portion and an enlarged terminal portion at one end thereof and integral therewith, said terminal portion being impregnated with metal throughout its respective cross-sectional area and having due to such impregnation a specific resistance which is lower than that of said heating portion, said heating portion and the axially inwardly directed radially extending wall of said enlarged terminal portion adjacent said heating portion carrying a material forming a protective coating thereon, a contact member disposed in axial abutment with the axially outwardly facing end of said enlarged terminal portion; and a tubular member of a length corresponding substantially at least to the thickness of said furnace wall for embracing said enlarged terminal portion and adjacent contact member to mount such portion and member in said furnace wall.

References Cited in the file of this patent

UNITED STATES PATENTS

50 1,553,379 Hellmund ----- Sept. 15, 1925

FOREIGN PATENTS

367,403 Great Britain ----- Feb. 18, 1932

409,031 Great Britain ----- Apr. 3, 1951

977,650 France ----- Apr. 3, 1951